

## UNITED STATES PATENT OFFICE

2,020,949

## ALLOY

Robert H. Leach, Fairfield, Conn., assignor to  
Handy & Harman, New York, N. Y., a corpora-  
tion of New York

No Drawing. Application November 6, 1934,  
Serial No. 751,710

## 7 Claims.

(Cl. 75—1)

This invention relates to alloys and is con-  
cerned more particularly with an alloy contain-  
ing silver, copper, and beryllium. The new alloy  
is capable of being given great hardness by suit-  
able heat treatment and because of that and its  
other physical characteristics, it may be used to  
advantage in different types of welding machines  
for electrode tips, contact points, etc.

The new alloy resembles that described and  
claimed in my Patent No. 1,928,429, September  
26, 1933, in that it contains the same ingredients,  
but it differs from the alloy of the patent in the  
respects that it contains less silver and more  
copper, and has different physical properties. By  
5 reason of the smaller proportion of silver, the  
new alloy can be made at a lower cost than the  
patented alloy. Also, it can be made consider-  
ably harder than the patented alloy by proper  
heat treatment. The new alloy has a somewhat  
lower electrical conductivity than the alloy of the  
patent, and thus the advantages of lower cost and  
greater hardness are to some extent counterbal-  
anced by the reduction in conductivity. But the  
conductivity of the new alloy is satisfactory for  
some purposes, and in those instances, its rela-  
tively low cost and its capacity for being given  
great hardness make its use highly desirable.

The new alloy contains silver ranging from 5%  
to 50%, beryllium ranging from 0.5% to 2.5%,  
30 and the remainder copper. Within these ranges,  
an increase in the amount of silver increases the  
electrical conductivity of the alloy while an in-  
crease in the amount of beryllium increases the  
capacity of the alloy to be hardened by proper  
35 treatment. Ordinarily, beryllium is present in an  
amount not less than .75% and preferably the  
amount does not exceed about 1.75% or 2%, since  
too great a proportion of the beryllium may make  
the alloy somewhat brittle. Where the use of the  
40 alloy is such that extreme hardness is desired and  
a tendency toward brittleness is not objectionable,  
the amount of beryllium employed may approach  
the upper limit.

In making the new alloy, the beryllium is pref-  
erably employed in the form of a master alloy  
45 containing silver or copper and about 10% to 12%  
or 13% beryllium. This master alloy is then  
combined with suitable amounts of silver and  
copper to produce the final alloy. The use of  
50 the master alloy is desirable since beryllium is

readily oxidized and at present is somewhat ex-  
pensive.

Examples of the new alloy which are suitable  
for commercial purposes are as follows, the  
analyses being approximate in each case:

## Example No. 1

|           | Per cent |
|-----------|----------|
| Silver    | 5        |
| Copper    | 93.8     |
| Beryllium | 1.2      |

## Example No. 2

|           | Per cent |
|-----------|----------|
| Silver    | 20       |
| Copper    | 78       |
| Beryllium | 15       |
|           | 2        |

## Example No. 3

|           | Per cent |
|-----------|----------|
| Silver    | 30       |
| Copper    | 68.25    |
| Beryllium | 20       |
|           | 1.75     |

The alloy of Example No. 1 may be considered  
as representative of a class, the members of which  
contain silver ranging from 5% to 20%, copper 25  
ranging from 78% to 94%, and beryllium ranging  
from 1% to 2.5%. Alloys in this class may be  
given a hardness which ranges from 100 to 112  
on the Rockwell "B" scale, depending on the com-  
position and the heat treatment, and their elec- 30  
trical conductivity varies from 30% to 35% of  
that of pure copper.

The alloy of Example No. 2 may be considered  
to be representative of a class, the members of  
which contain silver ranging from 20% to 40%, 35  
copper ranging from 58% to 78%, and beryllium  
ranging from 0.5% to 2.5%. Such alloys have a  
Rockwell "B" hardness of 68 to 112 and a conduc-  
tivity from 35% to 50% of that of pure copper,  
depending upon the percentages of the various 40  
ingredients and of the heat treatment to which  
the specific alloy is subjected. The alloy of Ex-  
ample No. 3 is another member of this class.

In addition to the classes above described, ex-  
amples of the new alloy may fall into a third 45  
class, the members of which contain silver rang-  
ing from 40% to 50%, copper ranging from 47.5%  
to 58%, and beryllium ranging from 0.5% to 2.5%.  
The members of this class have a Rockwell "B"  
hardness varying from 68 to 100 and a conductiv- 50

ity from 45% to 55% of that of pure copper, depending upon the composition and heat treatment.

The method of hardening the new alloy is similar to that described in my patent above mentioned. The alloy is first annealed for a substantial period of time and then instantly quenched. It is then heated for a further period of time at a lower temperature, a great increase in hardness resulting from the second heating. While the heating in both instances, is a function of both time and temperature, for many purposes, it is satisfactory to carry out the preliminary annealing by heating the alloy for a period of about two hours at a temperature ranging from about 1375° F. to 1400° F. Subjecting the alloy to such temperatures for the time mentioned appears to result in substantially complete solid solution. Following the quenching, further heating of the alloy gives the precipitation hardening effect. For some of the new alloys, I have found that the desired hardening may be obtained by heating for a period of about two hours at a temperature ranging from about 625° F. to about 650° F., although heating for a longer period may be required to obtain complete precipitation. Temperatures as high as 675° F. do not provide the same degree of hardening as the lower temperatures, but temperatures lower than 625° F. may be used, provided the heating is carried on for a longer time.

The heat treatment described imparts great

hardness to the alloy and the degree of hardness depends on the amount of beryllium present. For the same amount of beryllium and with heat treatment under the same conditions, the new alloy has a greater hardness than that of the 5 patent.

What I claim is:

1. An alloy consisting of silver in an amount ranging from about 5% to an amount exceeding 40% and substantially less than 50%, beryllium 10 in an amount ranging from about 0.5% to about 2.5%, and the remainder copper.

2. An alloy which consists of silver ranging from about 5% to about 20%, copper ranging from about 78% to about 94%, and beryllium 15 ranging from about 1% to about 2.5%.

3. An alloy which consists of silver ranging from about 20% to about 40%, copper ranging from about 58% to about 78%, and beryllium 20 ranging from about 0.5% to about 2.5%.

4. An alloy which consists of silver ranging from about 40% to an amount substantially less than 50%, copper ranging from about 47.5% to about 58%, and beryllium ranging from about 0.5% to about 2.5%.

5. An alloy which consists of about 5% silver, about 93.8% copper, and about 1.2% beryllium.

6. An alloy which consists of about 20% silver, about 78% copper, and about 2% beryllium.

7. An alloy which consists of about 30% silver, 30 about 68.25% copper, and about 1.75% beryllium.

ROBERT H. LEACH.